

Nov. 12, 1940.

L. J. HOLLMAN ET AL

2,221,350

FURNACE DOOR

Filed May 1, 1939

2 Sheets-Sheet 1

FIG. 1.



FIG. 2.



FIG. 3.



Inventors:

LEWIS J. HOLLMAN and  
WILLIAM F. NOEL.

by:

John E. Jackson  
their Attorney.

Nov. 12, 1940.

L. J. HOLLMAN ET AL

2,221,350

FURNACE DOOR

Filed May 1, 1939

2 Sheets-Sheet 2

FIG. 4.



FIG. 5.



Inventors:

LEWIS J. HOLLMAN and  
WILLIAM F. NOEL

by: *John E. Jackson*  
Their Attorney.

## UNITED STATES PATENT OFFICE

2,221,350

## FURNACE DOOR

Lewis J. Hollman, Munhall, and William F. Noel,  
Lincoln Place, Pa.

Application May 1, 1939, Serial No. 271,140

5 Claims. (Cl. 110—173)

The present invention relates to reenforced high temperature insulated linings for furnace doors, pit covers and the like.

An object of this invention is to provide a furnace door or pit cover construction which will not crack or spall when subjected to heating or cooling or to opening and closing.

A further object of the invention is to provide a door or cover which is easily repaired should it become crushed or bumped and a door in which cracks and crevices prevalent in doors of brick, refractory or insulating materials are eliminated.

Other objects and advantages will become apparent as the description proceeds and reference is had to the accompanying drawings, in which:

Figure 1 is a front elevation of a door constructed in accordance with the present invention;

Figure 2 is a section on line II—II of Figure 1;

Figure 3 is an enlarged section on line III—III of Figure 1;

Figure 4 is a section on line IV—IV of Figure 1; and,

Figure 5 is an enlarged detailed fragmentary section of Figure 4.

In the drawings, the reenforced high temperature lining is shown as applied to a prefabricated furnace door. The door which is illustrated as an example only, comprises a steel framework including top, bottom and side members 2 preferably angle iron members secured together in any conventional manner. Horizontal reenforcing members 3 extend between the side members 2, at spaced distances from the top to the bottom of the framework and are secured, in any conventional manner, to the frame members 2. Vertical reenforcing members 4 are secured, in any conventional manner, to the frame members 2 and the horizontal members 3. In addition, suitable diagonal reenforcing members 5 may be provided to form the completed framework. While the drawings illustrate a flat straight door or cover, it may be curved or fabricated to any shape to suit the face of the opening of the furnaces or pits with which it is to be used.

The framework having been fabricated, there is placed within the plane thereof, two layers of reenforcing steel mesh, the gage or weight of which may vary with the weight and size of the door or cover desired. The first layer of reenforcing wire mesh is illustrated at 6, and its position within the framework is governed by the thickness of the door or cover to be made. This wire mesh 6 is positioned substantially

parallel to the framework and preferably at a distance from the outer face thereof equal to about one-fourth of the thickness of the door or cover desired.

A second reenforcing wire mesh structure 7 is positioned within the framework preferably at a distance from the outer face thereof approximately equal to about one-half of the thickness of the door or cover.

Secured in any conventional manner to the inner sides of each of the top, bottom and side frame angle members 2, is a member 8 to which is secured, in any desired manner, an angle member 9, one arm being provided with an opening to receive the ends 10 of both the wire mesh 15 layers 6 and 7. This secures the layers of wire mesh to all parts of the framework and, to maintain the proper distance between the two wire mesh layers, there are provided the spacing wires or rods 12. The ends of said spacing rods 20 are twisted around or otherwise secured to the respective wire mesh layers. As a means for reenforcing that portion of the high temperature insulating material adjacent the surface exposed to the heat or inside face of the door or cover, 25 there are secured at spaced intervals to the wire mesh structure 7, a plurality of wires or rods 15 which are preferably twisted or distorted, which rods extend through about three-fourths of the thickness of the insulated part of the door or cover 30 between the reenforcing mesh 7 and the surface exposed to the heat or inside face of the door or cover.

The body of the door or cover, according to the present invention, is a high temperature resisting insulating material 14, which comprises approximately 48 per cent. by weight of a high temperature resistant insulating material which is crushed into irregular fragments from one-half to three-fourths of an inch in diameter, 24 per 40 cent. by weight of a similar material with said material being crushed to the extent that it will pass through a one-eighth inch square mesh, 24 per cent. by weight of a high temperature cement, and a sufficient quantity of water to thoroughly 45 mix said materials together into a plastic state. The plastic mortar is then carefully worked into the door or cover so that all spaces between the reenforcing mesh are properly filled and so that all of the reenforcing wires and rods are in proper 50 position as the door or cover is being filled to the proper thickness. The amounts and nature of the material used to make up the high temperature resistant insulated lining may be changed to suit the conditions of service re- 55

quired. After the door or cover has been built up to the required thickness, it is permitted to set until thoroughly dried before being put into use. When installed, the door must be slowly heated, so as to evaporate all moisture remaining therein, after which, the door will withstand the high temperatures without danger of cracking or spalling.

While we have shown and described a specific embodiment of the present invention, it will be seen that we do not wish to be limited exactly thereto, since various modifications may be made without departing from the scope of the invention, as defined by the following claims.

15. We claim:

1. A furnace door comprising a framework, at least two layers of wire mesh arranged within said framework substantially parallel to each other and to said framework and extending over 20 the entire area thereof, and a high temperature resisting refractory lining arranged on the inner side of said framework, said layers of wire mesh being attached to the framework and spaced apart from each other and being all embedded 25 in the refractory lining material for reenforcing the same.

2. A furnace door comprising a framework, at least two layers of wire mesh arranged within and attached to said framework substantially 30 parallel to each other and to said framework, and a high temperature resisting refractory lining arranged on the inner side of said framework, means for spacing said layers of wire mesh from each other, a plurality of twisted wires 35 carried by the inner layer of wire mesh and extending toward the inner side of said door, said layers of wire mesh, spacing means and inwardly extending twisted wires being all embedded in the refractory lining material for re-enforcing the same.

40. 3. A furnace door comprising a framework, two layers of wire mesh arranged within said framework substantially parallel to each other and to said framework, and a high temperature resisting refractory lining arranged on the inner side of said framework, one of said layers of wire mesh being positioned substantially cen-

trally of the thickness of the door with the other layer being positioned between the last mentioned layer of wire mesh and said framework, both of said layers of wire mesh being attached to said framework and embedded in said refractory lining material so as to reenforce the same.

4. A furnace door comprising a framework, two layers of wire mesh arranged within and attached to said framework substantially parallel 10 to each other and to said framework, and a high temperature resisting refractory lining arranged on the inner side of said framework, one of said layers of wire mesh being positioned at a distance from the outer face of said framework 15 equal to about one-fourth the thickness of the door with the other of said layers of wire mesh being positioned at a distance from the outer face of said frame equal to about one-half the thickness of the door, both of said layers of wire 20 mesh being embedded in said refractory lining material so as to reenforce the same.

5. In combination with a door to cover framework, two layers of wire mesh arranged within said framework substantially parallel to each 25 other and to said framework and connected thereto, a high temperature resisting refractory lining arranged on the inner side of said framework, one of said layers of wire mesh being positioned at a distance from the outer face of said frame equal to about one-fourth the thickness of the door with the other of said layers of wire mesh being positioned at a distance from the outer face of said frame equal to about one-half the thickness of the door so as to be positioned substantially in the center thereof, a plurality of wire members extending between said layers of wire mesh for spacing the same from each other, and a plurality of twisted wires carried by the 30 said centrally positioned layer of wire mesh and 35 extending toward the inner side of said door, said layers of wire mesh, spacing wires, and inwardly extending twisted wires reenforcing the refractory lining material in which they are embedded.

45. LEWIS J. HOLLMAN.  
WILLIAM F. NOEL.